

Patented June 29, 1926.

1,590,987

# UNITED STATES PATENT OFFICE.

GEORGE SIVOLA, OF DEXTER, NEW YORK.

## CHEMICAL PULP-COOKING PROCESS.

No Drawing.

Application filed December 4, 1925. Serial No. 73,270.

This invention relates to a new method of testing pulp from time to time during the cooking operation to enable the cook to properly control the cooking operation and also 5 the blowing point, as more fully hereinafter set forth.

In the methods at present in use, the cook keeps the temperature and pressure within certain limits which are adapted to each individual mill. He draws samples of the liquor from time to time and analyzes the same for total, free and combined  $\text{SO}_2$ ; smells it, and notes its appearance; then 10 judges the velocity with which the cellulose is liberated from the lignin by coloration of the liquor. From these facts he makes his deduction and operates the digester accordingly. The principal methods of determining the blowing point, i. e., the time when 15 the cooking is completed, are:

(a) *Acid test.*—The cook draws off a portion of the cooking liquor, tests for total  $\text{SO}_2$ , and blows the digester at a certain acid test.

(b) *Color and smell test.*—The cook takes a sample of the liquor, smells it, and tests the color of the liquor against a predetermined color standard, and when he finds that the liquor has become of standard color, 30 he blows off the digester.

(c) *Mitscherlich ammonia test.*—The cook takes a sample of the liquor, makes ammonia test to determine the amount of lime present at the latter part of the cooking, basing the 35 blowing point on the height and appearance of the precipitate and also on the color and smell of the liquor.

As outlined above, there are no standard methods for cooking, controlling and testing. They vary in different mills depending upon: first, the nature of the wood; second, the composition of the acid; third, the personal ideas of the man in charge. Thus, the blowing point of the digester by acid, color, 40 smell, etc., tests is more or less guess work, as they tell nothing about the quality of the pulp which is about to be blown. In the presence of so many variable factors, all of which more or less affect the product of the sulphite process, the blowing of two digesters consecutively are different in regard to bleach consumption and other qualities (strength, for instance) because: (a) The predetermined standards at certain stages of 45 the cooking seldom agree with the production obtained; (b) They are based more or

less on the liquor and not on the pulp itself.

It is the object of my invention to substitute for these indefinite ways of controlling the cooking and determining of the correct 60 blowing point a process which will eliminate indefiniteness by being based on the quality of the pulp itself. My process is based on the following facts: When a given weight of pulp (which is taken out of the 65 digester under pressure during the cooking period) is added to a definite volume of potassium permanganate ( $\text{KMnO}_4$ ) solution which is acidified with sulphuric acid ( $\text{H}_2\text{SO}_4$ ), the rate of absorption of the permanganate by the incrusting matters remaining in the pulp corresponds to the degree of disintegration of cellulose, the quickness of the reaction furnishing a measure of the delignification of the pulp that 70 can be expressed in seconds.

My tests are made from time to time, say a half hour or one hour apart, and for each test I proceed as follows: Take a sample of pulp from the digester through a valve, preferably a valve made especially for this purpose. Take a sample of acid and test for total  $\text{SO}_2$ . Disintegrate the pulp and wash it thoroughly, squeezing the water out by hand or wringer. Weigh off on fine scale a 80 portion of this pulp which corresponds to  $2\frac{1}{2}$  grams air-dry pulp. Take potassium permanganate ( $\text{KMnO}_4/100$ ); pour into colorless glass or tube with ground stopper, 85 200 to 300 cc.; then acidify it with 2 cc.  $\text{H}_2\text{SO}_4/1$ . Keep normal sulphuric acid ( $\text{H}_2\text{SO}_4/1$ ). Keep 90 temperature of permanganate same for each test, for example,  $25^\circ \text{C}$ .

I then carry out the test as follows: Take sample of the pulp, washed and disintegrated as described, in one hand; start stopwatch; drop the pulp into the solution; put stopper in tube or flask; start shaking gently and regularly, at the same time observing the color of the solution by the eye; 95 when color changes from initial color, namely, violet, to yellow (or yellowish brown), stop the watch; note in seconds the time required to decolorize the solution.

As soon as the pulp becomes soft enough to 100 disintegrate the chips as stated, I start testing by using the foregoing method. I make these tests at intervals of half an hour or an hour, and keep a record of each temperature as well as of each acid test. I decide 110 a uniform rate of increase in temperature to produce a desired quality of pulp and also

decide which kind of acid most economically produces the desired quality of pulp. I also work out a table, by observing which the cook can tell whether or not the cooking process is going correctly.

For a sample of a table, I have worked out the following for use in the cooking of ordinary hard pulp by the Mitscherlich process:

| Acid. | Pulp test.                |                      |
|-------|---------------------------|----------------------|
|       | Total $SO_2$<br>per cent. | Seconds at<br>25° C. |
| 10    | 0.90                      | 10                   |
|       | 0.80                      | 11                   |
| 15    | 0.70                      | 12                   |
|       | 0.64                      | 13                   |
|       | 0.58                      | 14                   |
|       | 0.54                      | 15                   |
|       | 0.51                      | 16                   |
|       | 0.48                      | 17                   |
| 20    | 0.45                      | 18                   |
|       | 0.41                      | 19                   |
|       | 0.38                      | 20                   |
|       | 0.35                      | 21                   |
|       | 0.32                      | 22                   |

The manner of using the foregoing table will be obvious from the following example: If the total  $SO_2$  were 0.54% and the pulp at the same time were 13, where it should be at least 15, this would show that the cooking process was not going correctly. In other words, it is relieving too much. So, by keeping close watch of the stock and acid test and observing the table, the cooking process can be corrected accordingly.

When the stock test shows that it has reached the point required to give the specified kind of pulp, the digester is ready to be blown. As far as the weight of pulp, and proportions of sulphuric acid and potassium permanganate are concerned, there are no definite ratios; they may vary indefinitely. For example, same weight of pulp, same volume of potassium permanganate, and greater volume of sulphuric acid would give different results than shown in the table, but the stock would be of the same hardness.

It will be observed that by reason of the fact that my tests are based on the pulp itself and not on the liquor, guess work is eliminated. It also makes it possible to produce any desired quality of pulp by working out a table and observing it, as previously described. It also makes it possible to know the exact time to blow off the digester. Also, it makes it possible to produce pulp which is practically uniform in hardness, strength, color, etc., this being one of the most important advantages of my method.

My method also enables me to obtain the highest yield by avoiding overcooking and knowing the exact blowing point. I also economize in sulphur consumption by reason of the high yield and because of the fact that I may determine the most economical composition of acid, it being known that the higher the blowing test for the acid, the greater the loss of sulphur. The higher yield

and the avoidance of overcooking and the blowing at the exactly proper point enable me also to produce lower steam consumption. My method also is time-saving in that the softer pulp I cook, the longer time it takes; for example, if "hard" pulp is desired, instead I get soft pulp under the present methods, thus wasting the time that was taken from the period when the pulp was of the desired quality. It necessarily follows that I get increase of production by reason of the higher yield, saving of time. It will be understood that for each particular purpose I can determine the most economical procedure. For example, if I am cooking easy bleaching pulp, I can determine the correct hardness and thus balance the yield, sulphur, steam consumption, time, etc., against the cost of bleaching, loss of yield, etc. It will also be obvious that my method is not confined to use of the chemicals mentioned above, but can be carried out with any chemicals which may be used for determining the degree of disintegration of the pulp sample in the above-described way, during the cooking period in any chemical pulp process.

What I claim as new is:

1. In chemical pulp cooking, the process of ascertaining the progress of the cooking operation, consisting in removing from the cooking mass a portion of the mass, subjecting a given weight of this separated pulp to the action of a definite volume of a chemical solution capable of reacting thereon in such manner as to cause a change in color of the solution, and observing and noting the time required for such chemical reaction to take place.

2. In chemical pulp cooking, the process of ascertaining the progress of the cooking operation, consisting in removing a portion of the pulp during the cooking operation, washing and disintegrating the pulp and removing the free water therefrom, taking a definite weight of this washed and disintegrated pulp and subjecting the same to the action of a given volume of a chemical solution capable of reacting on the pulp to change the color of the solution, and noting the time required for such change of color to take place.

3. In sulphite pulp cooking, the process of ascertaining the progress of the cooking operation, consisting in removing a part of the cooking liquor and testing the same for total  $SO_2$ , removing a part of the pulp at the same time and subjecting a given weight of this pulp to the action of a definite volume of a chemical solution capable of absorption by the incrusting matters remaining in the pulp and causing by this reaction a change in color of the solution, and noting the time required for this change in color to take place, the quickness of said reaction furnish-

ing a measure of the delignification of the pulp that can be expressed in seconds.

4. In chemical pulp cooking, the process of ascertaining the progress of the cooking operation, consisting in removing a portion of the pulp, disintegrating and washing the pulp, taking a given weight of this washed pulp separated from its free water and subjecting it to the chemical action of a

10 definite volume of potassium permanganate

( $\text{KMnO}_4$ ) acidified with sulphuric acid ( $\text{H}_2\text{SO}_4$ ), and noting the rate of absorption of the permanganate by the incrusting matters remaining in the pulp, this rate of absorption being an index of the degree of <sup>15</sup> disintegration of the cellulose.

In testimony whereof I hereunto affix my signature.

GEORGE SIVOLA.